

March 24, 1970

J. C. PETERSEN  
BONDED NONWOVEN SHEETS WITH A DEFINED  
DISTRIBUTION OF BOND STRENGTHS

3,502,538

Filed June 14, 1968

2 Sheets-Sheet 1

**FIG. 1**



**FIG. 2**



**FIG. 6**

BY

*Sol Schwartz*  
ATTORNEY

INVENTOR

JOSEPH CLAINE PETERSEN

March 24, 1970

J. C. PETERSEN  
BONDED NONWOVEN SHEETS WITH A DEFINED  
DISTRIBUTION OF BOND STRENGTHS

3,502,538

Filed June 14, 1968

2 Sheets-Sheet 2

**FIG. 3**



**FIG. 4**



**FIG. 5**



BY

*Sol Schwartz*  
ATTORNEY

3,502,538  
BONDED NONWOVEN SHEETS WITH A DEFINED  
DISTRIBUTION OF BOND STRENGTHS

Joseph Claine Petersen, Laramie, Wyo., assignor to E. I. du Pont de Nemours and Company, Wilmington, Del., a corporation of Delaware  
Continuation-in-part of abandoned application Ser. No. 390,020, Aug. 17, 1964. This application June 14, 1968, Ser. No. 747,405

Int. Cl. B32b 5/16

U.S. Cl. 161—150

8 Claims

## ABSTRACT OF THE DISCLOSURE

Bonded nonwoven sheets of defined bond parameters exhibit high tufted-grab-tensile strength and dye-beck-width stability. Such sheets contain matrix fibers having an average breaking strength of at least 7 grams and a multiplicity of bonds having a strength greater than 0.1 gram, the average strength of these bonds being at least 0.9 gram and less than the matrix fiber breaking strength, the bond strength distribution being characterized by a variance of at least 4, the number of bonds being such that the product of the number of bonds per cubic centimeter and the average bond strength is greater than  $5 \times 10^4$  g./cm.<sup>3</sup> and this product divided by the fiber breaking strength is less than  $9 \times 10^3$ /cm.<sup>3</sup>

## DETAILED DESCRIPTION OF THE INVENTION

This application is a continuation-in-part of my application Ser. No. 390,020, filed Aug. 17, 1964, now abandoned.

This invention relates to nonwoven sheet structures, in particular to bonded nonwoven sheets which have a combination of structural features that render such sheets particularly suitable as backings for tufted carpets.

Nonwoven sheet materials which are useful as primary backings for tufted carpets offer advantages over the known woven jute backings in such properties as dimensional stability, uniformity, supply stability, and hydrophobicity.

It has now been found that the number of bonds present in the nonwoven sheet materials and the bond strengths have a material effect on the characteristics necessary for primary backings. As the tufting needles penetrate the sheet, the fibers are displaced and they become aligned around the tufting yarns. Excessive fiber breakage occurs during this operation resulting in tufted carpets which are deficient in grab-tensile strength unless the bonds are weaker than the fibers. A very lightly bonded sheet, although permitting the fibers to move freely with a minimum of fiber breakage during the tufting operation lacks adequate sheet dimensional stability during subsequent processing. When tufted, the nonwoven sheet with too few self-bonds, undergoes shrinkage in the cross-machine direction during passage through the dye-beck.

It is a purpose of this invention to provide a nonwoven sheet material that is useful as a primary carpet backing.

It is another purpose of this invention to provide a carpet backing that can be made with comparative ease and which exhibits good tufted-grab-tensile strength and good dye-beck-width stability.

An additional purpose is to provide a nonwoven sheet which is less sensitive to damage by variations in the tufting needles such as burred, barbed, blunt, off-size, etc. needles.

Another purpose is to provide a nonwoven sheet having a combination of high tensile and tear strength.

These and other purposes of the invention are attained by providing a nonwoven sheet comprising synthetic organic fibers having an average breaking strength of at least 7 grams, bonded by a multiplicity of bonds with a bond strength greater than 0.1 gram. In the sheets, the average bond strength of these bonds is at least 0.9 gram and less than the fiber-breaking strength, the distribution of the strength of the bonds is characterized by a variance of at least 4, the number of bonds is such that the product of the number of bonds per cubic centimeter and the average bond strength is greater than  $5 \times 10^4$  g./cm.<sup>3</sup> and this product divided by the fiber-breaking strength is less than  $9 \times 10^3$ /cm.<sup>3</sup>

The invention will be further understood by reference to the drawings in which:

FIGURE 1 is a graph showing the relationship between dye-beck-width loss of tufted nonwoven sheets and the average bond strength ( $\bar{S}$ ) of the bonds in the untufted sheets;

FIGURE 2 is a graph showing the relationship between the dye-beck-width loss of tufted nonwoven sheets and the variance ( $\sigma^2$ ) in bond strength (as determined herein) in the untufted sheets;

FIGURE 3 is a graph showing the relationship between the dye-beck-width loss of tufted nonwoven sheets and the product ( $N_b \bar{S}$ ) of the number of bonds per cubic centimeter ( $N_b$ ) and the average bond strength in the untufted sheet;

FIGURE 4 is a graph showing the relationship between grab-tensile strength of the tufted nonwoven sheets and the product ( $N_b \bar{S}$ ) divided by the fiber-breaking strength ( $f$ ) in the untufted sheet;

FIGURE 5 is a typical stress-strain curve obtained in the determination of the individual bond strengths; and

FIGURE 6 is a schematic representation of a bonded sheet of the invention showing matrix fibers 1 and bonds 2.

The nonwoven sheets of this invention are composed of synthetic organic fibers which are bonded into a coherent structure. The bonds may comprise self-bonds and adhesive bonds, the latter being bonds between dissimilar materials. Considering only the bonds which have a bond strength of at least 0.1 gram, the average bond strength ( $\bar{S}$ ) must be at least 0.9 gram. This is the first criterion for acceptable performance of the nonwoven sheets of this invention as primary carpet backings. As indicated in FIGURE 1, an average bond strength below 0.9 gram leads to nonwoven sheets which, when tufted, exhibit excessive dye-beck-width losses. The upper limit on the average bond strength is the average fiber-breaking strength. Above this level the fibers rather than the bonds will break during tufting and this leads to a poor tufted-grab-tensile strength. The average bond strengths of preferred sheets of this invention will often be no more than about 40% of the minimum fiber breaking strength of 7 grams. Referring to FIGURE 1, it will be seen that Sample A has an average bond strength of 0.55 gram and gives a dye-beck-width loss of 26%, while Sample B, with an average bond strength of 1.2 grams, gives a low-dye-beck-width loss of 2.3%. The two samples have approximately the same number of bonds:  $6.95 \times 10^4$  bonds/cm.<sup>3</sup> for Sample A and  $5.85 \times 10^4$ /cm.<sup>3</sup> for Sample B.

A second criterion for acceptable performance of the nonwoven sheets of this invention as a primary carpet backing is that the distribution of strengths of the bonds must be such that the variance is greater than 4. As indicated in FIGURE 2, dye-beck-width losses increase rapidly below this level of variance. This is the type of behavior observed with an under-bonded sheet having a variance

below 4, that is, a narrow distribution of weak bonds. With overbonded sheets having a narrow distribution of very strong bonds and therefore a variance of less than 4, the tufted-grab-tensile is low. A broader distribution of bond strengths in the nonwoven sheets of this invention permits wide limits on average bond strengths and bond concentration to give good products. A narrow bond-strength-distribution product necessitates very narrow limits on the number of bonds thus requiring precise control of the bonding conditions. Certain products with a variance of bond-strength-distribution below 4 may, on occasion, give acceptable performance as primary carpet backings. Such products are sensitive to tufting needle condition and require precise control of finishing and tufting processes.

Variance, as used herein, has its accepted meaning in statistical analysis and is defined as follows:

$$\sigma^2 = \frac{\sum_{x=1}^{x=m} (\bar{S} - s_x)^2}{m - 1}$$

where:

$\sigma^2$  is the variance,

$\bar{S}$  is the arithmetic mean of the bond strengths,

$s_x$  is the measured value of the individual bond strengths,

and

$m$  is the number of measurements.

A third criterion for acceptable performance is a minimum value of the product of the number of bonds per cubic centimeter ( $N_b$ ) and the average bond strength. This product, which represents the total strength of the bonds in a cubic centimeter of the nonwoven sheet, must be at least  $5 \times 10^4$  g./cm.<sup>3</sup>. FIGURE 3 illustrates the sharp increase in dye-beck-width loss when the value of the product ( $N_b\bar{S}$ ) is less than  $5 \times 10^4$  g./cm.<sup>3</sup>. Thus, not only must average bond strength be above the minimum value of 0.9 gram, but also the bond concentration must be sufficient for the product  $N_b\bar{S}$  to satisfy the third criterion. The product is used rather than the bond concentration alone since the higher the average bond strength, the fewer bonds that are required.

A fourth criterion for acceptable performance of the nonwoven sheets of this invention involves the upper limit on the bond concentration, the lower limit having been defined by the third criterion. In setting this upper limit, it is necessary to consider the fiber-break strength ( $f$ ) in addition to the average bond strength, since a greater number of strong bonds can be tolerated with stronger fibers. It has been found that the product of the average bond strength and the bond concentration divided by the fiber-break strength, that is  $N_b\bar{S}/f$ , should not be greater than  $9 \times 10^3$ /cm.<sup>3</sup>. This is illustrated in FIGURE 4 where it is shown that tufted-grab-tensile strength rises markedly when the value of  $N_b\bar{S}/f$  is below  $9 \times 10^3$ /cm.<sup>3</sup>. Above this level, the tufted strength of non-woven sheets is markedly lower.

As indicated above, it is necessary in order consistently to obtain overall satisfactory performance of nonwoven sheets as primary carpet backings, that all four of the structural criteria defined above be met. With this structural definition of the requirements of satisfactory nonwoven sheet materials, those skilled in the art of production of non-woven sheets will recognize several methods which can be used for the manufacture of these products. For example, nonwoven webs of fibers which will have the desired fiber-breaking strength after bonding may be bonded by a combination of resinous binders, which combination, by virtue of differences in adhesive properties among the two or more bonders being used, will lead to bonds with the required distribution of bond strengths while maintaining the required level of average bond strength. Alternately the required distribution in bond strengths may be obtained by varying the size of the

bond sites over a sufficiently wide range with a single resinous binder giving the specified average bond strength level (greater than 0.9 gram but less than the fiber break strength). The bond concentration may be controlled by the quantities of binder material being used. The binder 5 may be applied in any of the methods known in the art. This includes application from dispersion or solution, as a granular or powdery material, or as binder fibers. If required these binders can be activated by application of heat in the known manner. These bonding methods and 10 also the known solvent-bonding and self-bonding techniques have not been used before to make products meeting the structural criteria of the products of this invention.

15 The nonwoven webs which are used to prepare the products of this invention can be produced by the standard techniques of the nonwoven art and can be composed of staple fibers, continuous filaments or combinations of the two. Preferred products are composed of continuous filaments having a random distribution throughout the sheet. Such materials having especially high tear and tensile strength and exhibiting isotropic properties can be made by the general procedure of British Patent 932,482 and are especially preferred for use in the nonwoven sheets of 20 this invention. The process described in this British patent involves an integrated spinning, orientation and laydown of the filaments to give a random nonwoven web which is essentially free from filament aggregates. In this process, the freshly spun filaments are electrostatically charged 25 and are then permitted to separate due to the applied electrostatic charge before web laydown. The type of filaments used in this invention are not critical and such synthetic organic fibers as the polyamides, such as poly(hexamethylene adipamide) and polycaproamide, polyesters such as 30 poly(ethylene terephthalate), polyhydrocarbons, such as linear polyethylene, and isotactic polypropylene, etc., are 35 suitable.

A particularly preferred sheet material of this invention is produced from nonwoven webs of fibers of oriented 40 isotactic polypropylene as the matrix fibers and unoriented or low-oriented isotactic polypropylene fibers as the binder material. By virtue of the lower degree of orientation in the binder fibers, they have a lower softening point than the matrix fibers. By choosing the proper bonding temperature, bonds comprising self-bonds between the matrix 45 fibers, self-bonds between the binder fibers, and inter-bonds between the matrix and binder fibers can be produced. Since these can have different bond strengths, the required variance in bond-strength distribution can be 50 readily obtained. However, because self-bonds between the matrix fibers are involved, it is necessary when practicing this method to operate the bonding step at a sufficiently high temperature to obtain some degree of self-bonding between the matrix fibers. This can be readily obtained since the softening point of the low-oriented binder fibers is usually only about 5-10° C. below that of the 55 more highly oriented fibers.

The binder fibers can be incorporated into the web as separate low-oriented fibers or as low-oriented segments of mixed-orientation fibers containing higher oriented segments as well. Either of these methods can 60 readily be adapted for use in the aforementioned process of British Patent 932,482 for the production of continuous-filament nonwoven sheets. Separate binder and matrix filaments can be produced by using two separate spinning and drawing machines and combining the filaments prior to or during web laydown. They can also be produced by splitting the thread line from the spinneret so that a part by-passes the drawing operation. Another 65 method involves the use of a spinneret with varying capillary geometry which produces filaments with varying responses to the drawing operation. Nonwoven webs of filaments with segments having different levels of orientation can be produced by pulsing the throughput of 70 polymer going to the drawing operation, by pulsing the 75

draw ratio in the drawing operation, or by variation of the drawing temperature. This latter method can be carried out by passing the filaments over a fluted feed roll in the drawing step. It has been found that these various techniques produce satisfactory mixed-orientation webs for use in producing the nonwoven sheets of this invention.

The use of fibers of mixed orientation in the webs does not necessarily result in a bonded nonwoven sheet which meets all four of the above-described structural criteria. To meet these criteria, it is necessary to carry out the bonding operation under controlled conditions. Bonding of mixed-orientation webs can be carried out with less critical temperature control than necessary with sheets prepared by self-bonding of like thermoplastic fibers. Thus a range of about 3° and preferably bonding within a range of 1° C. produces acceptable product. This wider latitude of operable bonding conditions is of great significance to the commercial manufacture of bonded nonwoven sheets, particularly for the wide widths required in primary carpet backing.

The nonwoven sheets of this invention which are designed for use as primary carpet backings will usually have a unit weight of 2 to 5 oz./yd.<sup>2</sup> (68 to 170 g./m.<sup>2</sup>) with a preferred weight of about 3 to 4 oz./yd.<sup>2</sup> (102 to 136 g./m.<sup>2</sup>). The denier of the matrix or high-orientation filaments in the nonwoven sheets will range from about 3 to 15 (0.3 to 1.7 tex) with the proviso that the denier must be adequate to give a fiber-break strength of at least 7 grams. Thus, filaments of isotactic polypropylene with a tenacity of 3 grams per denier would obviously have to be at least about 3 denier (0.22 tex). A preferred range for polypropylene filaments is 6 to 9 denier (0.67 to 1 tex) per filament. In selecting the denier of the matrix filaments, consideration must also be given to the possible loss in tenacity during the bonding operation. The fiber-breaking strength which is significant in the characterization of the nonwoven sheets of this invention is the strength of the matrix filaments in the bonded sheet.

A method which can be used to measure the average bond strength of the bonded nonwoven sheets of this invention is described below. A sample of the bonded nonwoven sheet (2 in. x 0.125 in.) (5 cm. x 0.32 cm.) is delaminated in its thickness dimension into as many layers as can be obtained without distortion or tearing of the individual strips. The number of layers obtained will vary with the thickness of the product being tested but will usually be between 3 and 10. The purpose of delaminating and using narrow samples is to obtain layers having a limited but representative number of bonds so that in the subsequent tensile test, individual bond breakage can be followed and the likelihood of multiple bonds breaking simultaneously is minimized. Each of the delaminated layers is pulled apart in an Instron Tensile Tester using a 1-in. (2.5 cm.) jaw separation and a strain rate of 0.02 in. (0.05 cm.) per minute. The instrument is calibrated to 40 grams full scale, thus permitting readings down to 0.1 gram. Bonds having strengths less than 0.1 gram are not measured. A typical curve is shown in FIGURE 5. The drops in load, labeled S<sub>1</sub>, S<sub>2</sub>, etc., in the figure, after the maximum stress (F<sub>m</sub>) is reached are attributed to breakage of individual bonds.

As a delaminated layer is elongated, the resultant stress (F) is distributed over the bonds supporting the stress in the strip. At any section along the layer, the stress (F) will be distributed among the bonds supporting stress within that section. The stress potential of such section will be determined by the product of the number of bonds (N<sub>b</sub>) supporting the stress and their average strength ( $\bar{S}$ ). When the force on the layer exceeds the value of N<sub>b</sub>S for the weakest section of the layer, it will begin to fail at that point, and bonds in that section will begin to break. At higher elongations, the layer is held together by a few fibers and on continued elongation,

bonds are broken in sections further back and outside the original section of the bond breakage. This expanding area of bond breakage is not definable and some basis is needed to limit the bond-strength measurement to some small finite section which can be measured. The proper amount of elongation is determined from the maximum stress recorded (F<sub>m</sub>) which is equal to N<sub>b</sub>S for the section of the layer which breaks. Accordingly, the layer is elongated until the value of N<sub>b</sub>S and F<sub>m</sub> give the required agreement.

The section bond breakage is determined by taking photomicrographs of the delaminated layers before and after the bond-breaking test, comparing the same and measuring the area of disruption. This is the area that does not retain intact as seen from the comparison of the before and after photomicrographs. The thickness of the original sample can be readily measured by known methods, for example with an Ames gauge. From the area of bond breakage and the thickness of the original nonwoven sheet sample, the total volume, i.e. the section, of the sample in which the bond breakage occurred can be calculated.

In addition to the bonds in the individual delaminated layers, it is necessary to obtain a measure of the bonds broken in obtaining the delaminated layers. A measure of these bonds is obtained by delaminating the samples on the Instron Tensile Tester at a strain rate of 0.05 in./min. (0.127 cm./min.) and noting the number and strength of the bonds broken over an area equal to that affected in the above tensile test. This number is then multiplied by the number of delaminations used to obtain the specimens for the tensile test. The average bond strength, number of bonds, and the variance of the bond-strength distribution are calculated from the bond strengths measured on all the delaminated layers as well as those measured during delamination. From the area of bond breakage, the thickness of the sample, and the number of bonds which have been broken, the number of bonds per cubic centimeter can be calculated.

The machine direction tongue tear strength (TTT) of a tufted nonwoven fabric for all examples but Example XIV was measured in the following manner. A nonwoven fabric tufted as in Example II is cut into a sample 3 inches wide (cross-machine direction, across tufting rows) and 8 inches long (machine direction, along tufting rows). The TTT of Example XIV was determined on a 6 inch by 8 inch sample. The sample is cut in the center of the width 4 inches in the machine (tufting) direction. The sample is mounted in an "Instron" tester using 1.5 inch by 2 inch serrated clamps. With a jaw separation of 3 inches, one side of the sample cut is mounted in the upper jaw and the other side of the sample cut is mounted in the lower jaw. The sample is uniformly spaced between the jaws. The full scale load is adjusted to a value greater than the tear strength expected for the sample. Using a crosshead speed of 12 inches per minute and a chart speed of 10 inches per minute, the "Instron" is started and the sample is torn. An average of the three highest stresses (one hundred units=full scale deflection) during tearing is taken. If it is not possible to obtain three peaks, the average of the peaks obtained is taken. The tongue tear strength in pounds is the average highest stress divided by 100 and multiplied by the full scale load.

The "tufted grab tensile" of a nonwoven fabric was measured in the following manner. A sample tufted as in Example II is cut into samples 4 inches wide by 6 inches long in the tufting direction. The sample is mounted in an "Instron" using a 1 inch by 2 inch clamp on the back side and a 1 inch square clamp in the front side at a jaw separation of 3 inches. A crosshead speed of 12 inches per minute is used. The peak of the "Instron" curve is read and reported as pounds breaking strength.

The invention will be further illustrated by the following examples.

## EXAMPLE 1

Two nonwoven webs of 14% low-oriented and 86% high-oriented, isotactic polypropylene filaments are bonded under different process conditions to produce two bonded sheets 1A and 1B. The high-oriented polypropylene filaments are drawn 3.5 $\times$  after spinning from a polymer having a melt flow rate (MFR) (ASTM method D1238 at 230° C. with a loading of 2.16 kg.) of 12. They are 7.48 denier (0.38 tex) per filament and have a tenacity of 4.03 g.p.d. The low-oriented polypropylene filaments are drawn 1.21 $\times$  after spinning from a polymer having a MFR of 12. They are 7.73 denier (0.86 tex) per filament and have a tenacity of 1.62 g.p.d.

The webs are prepared as follows: 86% of the polypropylene filaments are spun through a 30-hole spinneret at a rate of 18 g./min. total. Fourteen percent of the polypropylene filaments are spun through a 5-hole spinneret at a rate of 3 g./min. total. Each spinneret hole for both spinnerets is 0.015 inch (0.038 cm.) in diameter. The temperature of the 30-hole spinneret is 242° C. and the 5-hole spinneret, 220° C. The filaments from the 30-hole spinneret are led around a heated feed roll operating with a surface temperature of 118° C., and advanced by means of an idler roll canted with respect to the heated roll. A total of 5 wraps is used on the heated feed roll, which is operated with a surface speed of 243 yd./min. (222 m./min.). The filaments leaving the heated feed roll are then passed 5 wraps around an idler roll/draw roll system operating cold with a surface speed of 858 yd./min. (785 m./min.). The filaments from the 5-hole spinneret are led to a heated roll operating with a surface temperature of 95° C., and a surface speed of 703 yd./min. (642 m./min.). The filaments are in contact with the heated roll for 180°. The filaments leaving the heated roll are then passed to a draw roll operating cold with a surface speed of 852 yd./min. (779 m./min.). The filaments are in contact with the draw roll for 180°. The filaments from both spinnerets meet and are guided so the low-oriented filaments are dispersed uniformly throughout the high-oriented filaments. The filaments are then electrostatically charged with a corona discharge device, passed into a draw jet and subsequently deposited on a moving belt to form a nonwoven web of randomly distributed continuous filaments. Two sections are cut from this product to constitute the filamentary webs to be bonded as indicated below.

Each of the filamentary webs is bonded by passing the web at a speed of 10 yd./min. (9 m./min.) while under restraint between one porous metal plate and one solid plate, each faced with cloth, for a distance of 37 inches (94 cm.) through a steam chamber in which saturated steam is maintained at superatmospheric pressure. The bonded sheets are prepared for tufting by the application of a lubricant in the following manner. The bonded sheets are submerged in a 4% aqueous dispersion of a polysiloxane which also contains 0.4% of a surface active agent (sodium alkylarylsulfonate). The sheets are then squeezed between two rolls with a nip pressure of 50 p.s.i.g. (3.5 kg./cm.<sup>2</sup>) at a speed of 1.5 yd./min. (1.4 m./min.) and dried in a circulating hot air oven for 45 minutes at a temperature of 93° C. The sheets are then tufted at the following conditions:

Gauge (distance between needles)—0.188 in.

Speed—400 tufts/min., 7 tufts/in.

Pile yarn—3700 denier (410 tex) continuous filament nylon

Tuft height—0.438 in.

Type pile—loop.

Details of bonding the webs and characterization of the bonded sheets including the properties of the tufted sheets appear in Table 1. Both sheets exhibit substantial grab tensile strength. Sheet 1A is underbonded and the values for variance and the product  $N_b\bar{S}$  are outside the

limits required for acceptable performance. The tufted sheet exhibits an unsatisfactory dye-beck-width loss. Sheet 1B is an example of a nonwoven sheet of this invention.

TABLE 1

|    |                                                                | 1A   | 1B   |
|----|----------------------------------------------------------------|------|------|
| 5  | Unit weight, oz./yd. <sup>2</sup>                              | 4.00 | 3.84 |
|    | Bonding conditions:                                            |      |      |
|    | Saturated steam pressure, p.s.i.a.                             | 66   | 75   |
|    | Bonding contact time, secs.                                    | 6.2  | 6.2  |
|    | Restraint on web, lb./in. <sup>2</sup> /oz./yd. <sup>2</sup>   | 0.75 | 0.75 |
| 10 | Characteristics of bonded sheets:                              |      |      |
|    | Average bond strength ( $\bar{S}$ ), grams                     | 0.98 | 1.13 |
|    | Variance ( $\sigma^2$ )                                        | 2.75 | 5.35 |
|    | No. bonds/cm. <sup>3</sup> $\times$ $\bar{S}$ ( $N_b\bar{S}$ ) | (1)  | (2)  |
|    | Fiber-breaking strength ( $f$ ), grams                         | 24.2 | 24.0 |
|    | $N_b\bar{S}/f$                                                 | (3)  | (4)  |
| 15 | Properties of tufted sheets:                                   |      |      |
|    | Grab tensile, lb.                                              | 164  | 133  |
|    | Dye-beck-width loss, percent                                   | 22   | 3.8  |
|    | Tongue tear (lbs.)                                             | 60   | 40   |

<sup>1</sup>  $3.42 \times 10^4$  g./cm.<sup>3</sup>

<sup>2</sup>  $11.5 \times 10^4$  g./cm.<sup>3</sup>

<sup>3</sup>  $1.4 \times 10^3$  cm.<sup>3</sup>

<sup>4</sup>  $4.79 \times 10^3$  cm.<sup>3</sup>

## EXAMPLE 2

A nonwoven web of 14% low-oriented and 86% high-oriented, isotactic polypropylene filaments is heated to produce a bonded sheet. The high-oriented polypropylene filaments are drawn 4.0 $\times$  after spinning from a polymer having a MFR of 12. They are 7.5 denier (0.83 tex) per filament and have a tenacity of 4.20 g.p.d. The low-oriented polypropylene filaments used remain undrawn after spinning from a polymer having a MFR of 12. The filaments are 8.0 denier (0.89 tex) per filament and have a tenacity of 1.5 g.p.d. The webs are prepared as follows: 86% of the polypropylene filaments are spun through a 30-hole spinneret at a rate of 18 g./min. total. 14% of the polypropylene filaments are spun through a 5-hole spinneret at a rate of 3 g./min. total. Each spinneret hole for both spinnerets is 0.015 inch (0.038 cm.) in diameter and the temperature of the 30-hole spinneret is 230° C. and the 5-hole spinneret, 224° C. The filaments from the 30-hole spinneret are led around a heated feed roll operating with a surface temperature of 118° C., and advanced by means of an idler roll canted with respect to the heated roll. A total of 5 wraps is used on the heated feed roll, which is operated with a surface speed of 227 yd./min. (207 m./min.). The filaments leaving the heated feed roll are then passed 5 wraps around an idler roll/draw roll system operating cold with a surface speed of 900 yd./min. (823 m./min.). The filaments from the 5-hole spinneret are led to one cold roll operating with a surface speed of 660 yd./min. (604 m./min.). The filaments are in contact with the roll for 270°.

The filaments from the spinnerets are combined and then laid down as a nonwoven web as in Example 1. The filamentary web is bonded as in Example 1 with saturated steam at a pressure of 95 p.s.i.a. (6.7 kg./cm.<sup>2</sup>). Properties of the bonded and tufted sheet are summarized in Table 2. The bonded sheet is lubricated and tufted as in Example 1.

TABLE 2

|                                  |                                                                   |                                        |
|----------------------------------|-------------------------------------------------------------------|----------------------------------------|
| 60                               | Unit Weight, oz./yd. <sup>2</sup> (g./m. <sup>2</sup> )           | 4.10 (139)                             |
| Characteristics of bonded sheet: |                                                                   |                                        |
|                                  | Average bond strength ( $\bar{S}$ )                               | —2.41 g.                               |
|                                  | Variance ( $\sigma^2$ )                                           | —29.3                                  |
| 65                               | No. of bonds/cm. <sup>3</sup> $\times$ $\bar{S}$ ( $N_b\bar{S}$ ) | $56.1 \times 10^4$ g./cm. <sup>3</sup> |
|                                  | Fiber-breaking strength ( $f$ )                                   | —17.3 g.                               |
|                                  | $N_b\bar{S}/f$                                                    | $32.4 \times 10^3$ cm. <sup>3</sup>    |
| Properties of Tufted Sheets:     |                                                                   |                                        |
|                                  | Grab-Tensile, lb. (kg.)                                           | —42 (19)                               |
|                                  | Dye-Beck-Width Loss                                               | —0%                                    |

This bonded sheet is heavily overbonded and, after tufting, exhibits very poor grab-tensile strength. The only criterion for acceptable performance which the bonded sheet does not meet is the maximum value of  $N_b\bar{S}/f$ .

**9**  
**EXAMPLE 3**

Two nonwoven webs of continuous, isotactic polypropylene filaments are prepared in the same general manner as that described in Example 2, except that the draw ratio of the highly drawn filaments is varied. Identification of the variables is made in Table 3. Prior to tufting, the sheets are lubricated as described in Example 1. The tufted sheet of Sample 3A has a good balance of grab-tensile strength and dye-beck-width loss. Sample 3B has high dye-beck-width loss at the same tensile value. These values and the characteristics of the bonded webs are shown in Table 4.

TABLE 3

| Sample  | High-Oriented Filaments |                       |            |                 |           |      | Low-Oriented Filaments |                 |           |      |                             |     |      |    |
|---------|-------------------------|-----------------------|------------|-----------------|-----------|------|------------------------|-----------------|-----------|------|-----------------------------|-----|------|----|
|         | Feed Speed<br>yd./min.  | Draw Speed<br>m./min. | Draw Ratio | Ten.,<br>g.p.d. | Den./Fil. | Tex. | Roll Speed<br>yd./min. | Den.,<br>g.p.d. | Den./Fil. | Tex. | Bond<br>Press.,<br>p.s.i.a. |     |      |    |
| 3A----- | 243                     | 222                   | 901        | 824             | 3.7       | 3.5  | 7.4                    | 0.82            | 660       | 604  | 1.56                        | 8.8 | 0.98 | 70 |
| 3B----- | 352                     | 322                   | 764        | 699             | 2.2       | 2.38 | 9.2                    | 1.02            | 660       | 604  | 1.38                        | 9.9 | 1.10 | 59 |

Three nonwoven webs of continuous, isotactic polypropylene filaments are prepared in the same general manner as that described in Example 1, except that the amount of low-oriented polypropylene filaments is varied by changing the number of those filaments, while keeping the number of high-oriented filaments constant. Identification of variables is made in Table 7. Prior to tufting, the bonded sheets are lubricated as described in Example 1. The tufted sheets of samples 5A and 5B have a good bal-

TABLE 3

| Sample  | High-Oriented Filaments |                       |            |                 |           |      | Low-Oriented Filaments |                 |           |      |                             |     |      |    |
|---------|-------------------------|-----------------------|------------|-----------------|-----------|------|------------------------|-----------------|-----------|------|-----------------------------|-----|------|----|
|         | Feed Speed<br>yd./min.  | Draw Speed<br>m./min. | Draw Ratio | Ten.,<br>g.p.d. | Den./Fil. | Tex. | Roll Speed<br>yd./min. | Den.,<br>g.p.d. | Den./Fil. | Tex. | Bond<br>Press.,<br>p.s.i.a. |     |      |    |
| 3A----- | 243                     | 222                   | 901        | 824             | 3.7       | 3.5  | 7.4                    | 0.82            | 660       | 604  | 1.56                        | 8.8 | 0.98 | 70 |
| 3B----- | 352                     | 322                   | 764        | 699             | 2.2       | 2.38 | 9.2                    | 1.02            | 660       | 604  | 1.38                        | 9.9 | 1.10 | 59 |

TABLE 4

| Sample  | Unit Weight          |                    |           |            | Tufted-Grab-Tensile      |      |                             |     | Dye-Beck-Width Loss, Percent |     |
|---------|----------------------|--------------------|-----------|------------|--------------------------|------|-----------------------------|-----|------------------------------|-----|
|         | oz./yd. <sup>2</sup> | g./m. <sup>2</sup> | $\bar{S}$ | $\sigma^2$ | N <sub>b</sub> $\bar{S}$ | f    | N <sub>b</sub> $\bar{S}$ /f | lb. | kg.                          |     |
| 3A----- | 3.75                 | 127                | 1.36      | 4.93       | 6.46 $\times 10^4$       | 23.3 | 2.77 $\times 10^3$          | 138 | 63                           | 2.3 |
| 3B----- | 4.04                 | 137                | 0.35      | 0.14       | 0.54 $\times 10^4$       | 17.7 | 0.30 $\times 10^3$          | 134 | 61                           | 2   |

**EXAMPLE 4**

Three nonwoven webs of continuous, isotactic polypropylene filaments are prepared in the same general manner as in Example 1 except that the draw ratio of the low-oriented filaments is varied. Identification of the variables is made in Table 5. Prior to tufting, the bonded sheets are lubricated as described in Example 1. The three bonded sheets meet all four structural criteria of the products of this invention. These values and the properties of the tufted sheets are shown in Table 6. The TTT values for Samples 4A and 4B are 38 and 37 respectively.

ance of grab-tensile and dye-beck-width loss. Sample 5C has high dye-beck-width loss at the same tensile value. These properties and the structural characteristics of the bonded sheets are summarized in Table 8.

35

TABLE 7

| Sample  | Weight percent<br>Low-oriented<br>Filaments | Bonding<br>Pressure,<br>p.s.i.a. | Unit<br>Weight,<br>oz./yd. <sup>2</sup> |
|---------|---------------------------------------------|----------------------------------|-----------------------------------------|
| 5A----- | 5                                           | 84                               | 3.45                                    |
| 5B----- | 25                                          | 74                               | 3.93                                    |
| 5C----- | 50                                          | 62                               | 3.46                                    |

TABLE 5

| Sample  | High-Oriented Filaments  |                          |               |                 |           |      | Low-Oriented Filaments   |                          |               |                 |           |      |    |
|---------|--------------------------|--------------------------|---------------|-----------------|-----------|------|--------------------------|--------------------------|---------------|-----------------|-----------|------|----|
|         | Feed<br>Speed,<br>y.p.m. | Draw<br>Speed,<br>y.p.m. | Draw<br>Ratio | Ten.,<br>g.p.d. | Den./Fil. | Tex. | Feed<br>Speed,<br>y.p.m. | Draw<br>Speed,<br>y.p.m. | Draw<br>Ratio | Ten.,<br>g.p.d. | Den./Fil. | Tex. |    |
| 4A----- | 244                      | 858                      | 3.5           | 4.00            | 8.3       | 0.92 | 263                      | 852                      | 3.2           | 3.68            | 8.5       | 0.94 | 86 |
| 4B----- | 235                      | 858                      | 3.6           | 4.10            | 8.0       | 0.89 | 320                      | 852                      | 2.7           | 3.0             | 8.0       | 0.89 | 89 |
| 4C----- | 223                      | 858                      | 3.8           | 4.30            | 7.4       | 0.82 | 466                      | 852                      | 1.8           | 2.12            | 8.4       | 0.93 | 81 |

TABLE 6

| Sample  | Unit<br>Weight,<br>oz./yd. <sup>2</sup> | $\bar{S}$ | $\sigma^2$ | N <sub>b</sub> $\bar{S}$ | f    | Tufted-Grab-Tensile, lb. | Dye-Beck-Width Loss, Percent |     |
|---------|-----------------------------------------|-----------|------------|--------------------------|------|--------------------------|------------------------------|-----|
| 4A----- | 4.14                                    | 1.23      | 7.25       | 11.8 $\times 10^4$       | 24.4 | 4.83 $\times 10^3$       | 145                          | 5.5 |
| 4B----- | 4.25                                    | 1.50      | 9.45       | 17.3 $\times 10^4$       | 24.9 | 6.95 $\times 10^3$       | 123                          | 4.3 |
| 4C----- | 4.03                                    | 1.41      | 6.71       | 10.7 $\times 10^4$       | 32.1 | 4.64 $\times 10^3$       | 155                          | 3.8 |

TABLE 8

| Sample  | $\bar{S}$ | $\sigma^2$ | N <sub>b</sub> $\bar{S}$ | f    | Tufted-Grab-Tensile, lb. | Dye-Beck-Width Loss, Percent | TTT |    |
|---------|-----------|------------|--------------------------|------|--------------------------|------------------------------|-----|----|
| 5A----- | 1.49      | 4.73       | 12.0 $\times 10^4$       | 23.3 | 5.15 $\times 10^3$       | 107                          | 3.8 | 37 |
| 5B----- | 1.41      | 11.8       | 9.28 $\times 10^4$       | 23.0 | 4.03 $\times 10^3$       | 150                          | 4.0 | 50 |
| 5C----- | 0.68      | 1.66       | 2.39 $\times 10^4$       | 21.2 | 1.13 $\times 10^3$       | 114                          | 32  | 44 |

**11**  
**EXAMPLE 6**

A nonwoven web of mixed-orientation polypropylene filaments is prepared as follows: polypropylene having a MFR of 12 is spun through a 30-hole spinneret at a total rate of 18 g./min. Twenty-seven spinneret holes are 0.015 in. (0.038 cm.) in diameter and 3 are 0.018 in. (0.046 cm.) in diameter. The temperature of the spinneret is 219° C. The filaments are led around a heated feed roll operating with a surface temperature of 114° C., and advanced by means of an idler roll canted with respect to the heated roll. A total of 5 wraps is used on the heated feed roll, which is operated with a surface speed of 207 yd./min. (189 m./min.). The filaments leaving the heated feed roll are then passed 5 wraps around an idler roll/draw roll system operating cold with a surface speed of 900 yd./min. (823 m./min.). The group of 27 filaments has a denier of 7.2 (0.8 tex) and a tenacity of 4.14 g.p.d., while the group of 3 filaments has a denier of 11.7 (1.3 tex) and a tenacity of 3.46 g.p.d.

The drawn filaments are electrostatically charged with a corona discharge device, passed into a draw jet, and subsequently deposited on a moving belt to form a nonwoven web of randomly distributed continuous filaments. The filamentary web is bonded as in Example 1 with saturated steam at a pressure of 99 p.s.i.a. (7.0 kg./cm.<sup>2</sup>). Prior to tufting, the bonded sheet is lubricated as in Example 1. The sheet characteristics and the tufted-sheet properties are summarized in Table 9. This example indicates that spinnerets with varying hole sizes can be used to prepare polypropylene filaments with different levels of orientation.

**EXAMPLE 7**

A nonwoven web is prepared with oriented polypropylene filaments having low-oriented sections along the fiber length. The polypropylene filaments are 7.02 denier (0.78 tex) per filament and have a tenacity of 4.11 g.p.d. in the high-oriented sections, and are 15.5 denier (1.7 tex) per filament and have a tenacity of 1.81 g.p.d. in the low-oriented sections. The high-oriented segments are about 18 in. (46 cm.) long and the low-oriented segments are about 2 in. (5 cm.) long. The web is prepared as follows: Polypropylene filaments are spun through a 30-hole spinneret at a rate of 18 g./min. total. Each spinneret hole is 0.015 in. (0.038 cm.) in diameter and the temperature of the spinneret is 235° C. The filaments are led to a heated feed roll having a circumference of 18.75 in. (47.7 cm.) with three 1.25 in. (3.17 cm.) grooves cut out 120° apart. The filaments are in contact with the roll for 220°. The surface temperature of the roll is 130° C. The roll is operated with a surface speed of 243 yd./min. (222 m./min.). The filaments leaving the heated feed roll are then passed 3 wraps around an idler roll/draw roll system operating cold with a surface speed of 858 yd./min. (784 m./min.). The filaments are then laid down as nonwoven web of randomly distributed continuous filaments as in Example 1.

The filamentary web is bonded as in Example 1 with saturated steam at a pressure of 70 p.s.i.a. (4.9 kg./cm.<sup>2</sup>). The bonded sheet is lubricated and then tufted by the procedure of Example 1. The sheet characteristics and the tufted-sheet properties are summarized in Table 9. The bonded sheet of this example has an excellent balance of tufted-grab-tensile strength and dye-beck-width loss.

**12**  
**EXAMPLE 8**

A nonwoven web of 14% (by weight) low-oriented and 86% high-oriented poly(ethylene terephthalate) filaments is prepared as follows: poly(ethylene terephthalate) (relative viscosity, 25.7) is spun through a 10-hole spinneret at a rate of 21 g./min. total and through a 4-hole spinneret at a rate of 3.44 g./min. total. The holes in both spinnerets are 0.004 in. (0.010 cm.) in diameter and the temperature of both spinnerets is 286° C. The filaments from the 10-hole spinneret are led to a pair of canted, cold feed rolls. One wrap is used on the feed rolls, which are operated with a surface speed of 1030 yd./min. (942 m./min.). The filaments leaving the feed rolls are then passed one wrap around a pair of canted draw rolls operating cold with a surface speed of 4,350 yd./min. (3,790 m./min.). These high-oriented filaments are 5.2 denier (0.58 tex) and have a tenacity of 4.37 g.p.d. The filaments from the 4-hole spinneret by-pass the roll system and are individually separated by Al Si Mag pins. These filaments are 5.3 denier (0.59 tex) and have a tenacity of 1.60 g.p.d. The filaments from both spinnerets meet and are then electrostatically charged with a corona discharge device, passed into a draw jet, and subsequently deposited on a moving belt to form a nonwoven web of randomly distributed, continuous filaments. The filamentary web is consolidated by passing the web supported on a leader cloth between two rolls at a speed of 0.225 yd./min. (0.206 m./min.). The top roll is covered with a 300-mesh screen and heated to a surface temperature of 105° C. The web is then bonded by passing it at a speed of 2.67 yd./min. (2.44 m./min.) while under low restraint between two polytetrafluoroethylene-coated 30-mesh screens for a distance of 24 in. (61 cm.) through a heated air chamber at 246° C. The bonded sheet is lubricated and tufted as described in Example 1. The sheet characteristics and the tufted-sheet properties are summarized in Table 9. The value of  $N_b\bar{S}/f$  for the sheet indicates that it is overbonded. This is in accord with the observed tufted-grab-tensile strength. The break strength of fibers in the bonded sheet is relatively low and this can at least partially explain both the high value of  $N_b\bar{S}/f$  and the low tufted-grab-tensile strength. The results in this example illustrate the importance of utilizing the breaking strength of the fiber in the nonwoven sheet after bonding in the calculation of  $N_b\bar{S}/f$ . Before bonding, the high-oriented filaments have a fiber-breaking strength of 22.7 g. (5.2 d.p.f.  $\times$  4.37 g.p.d.). Use of this figure in the calculation leads to a value of  $6 \times 10^3$  cm.<sup>3</sup> for  $N_b\bar{S}/f$  which is within the limits required for acceptable performance. The high temperature used for bonding appears to have caused some deorientation of the high-oriented filaments with a resulting loss in tenacity and the formation of a sheet which is overbonded for the level of fiber-breaking strength remaining after bonding.

**EXAMPLES 9-11**

The procedures of Example 8 are followed except that bonding in the heated air chamber is carried out at 241° C. for Example 9, at 238° C. for Example 10 and at 193° C. for Example 11. Of these, only the product of Example 9 falls within the scope of the present invention. Note the high dye-beck-width loss of the products of Examples 10 and 11. (See Table 9.)

TABLE 9

| Bonded Sheet | oz./yd. <sup>2</sup> | $\bar{S}$ | $\sigma^2$ | $N_b\bar{S}$       | $f$   | $N_b\bar{S}/f$     | Tufted-Grab-Tensile, lb. | Dye-Beck-Width Loss, percent |
|--------------|----------------------|-----------|------------|--------------------|-------|--------------------|--------------------------|------------------------------|
| Ex. 6-----   | 4.12                 | 1.21      | 8.4        | $15.4 \times 10^4$ | 21.5  | $7.1 \times 10^3$  | 95                       | 1.3                          |
| Ex. 7-----   | 4.11                 | 1.95      | 17.3       | $7.51 \times 10^4$ | 25.7  | $2.92 \times 10^3$ | 185                      | 3.5                          |
| Ex. 8-----   | 4.26                 | 1.83      | 5.64       | $13.5 \times 10^4$ | 9.2   | $14.7 \times 10^3$ | 81                       | 3.5                          |
| Ex. 9-----   | 4.28                 | 2.0       | 6.7        | $12.8 \times 10^4$ | 20.9  | $6.2 \times 10^3$  | 100                      | 5.0                          |
| Ex. 10-----  | 4.33                 | 0.88      | 1.4        | $3.4 \times 10^4$  | ----- | $1.6 \times 10^3$  | 153                      | 16                           |
| Ex. 11-----  | 3.88                 | 0.65      | 0.47       | $1.1 \times 10^4$  | ----- | $0.5 \times 10^3$  | 132                      | 38                           |

<sup>a</sup> Estimated.

NOTE.—TTT values for Examples 6, 7, 8, 9, 10, and 11 are 31, 50, 21, 30, 42 and 43 respectively.

The graphs in FIGURES 1, 2, 3, and 4 are based on the data obtained in Examples 1-8, and additional cumulative data obtained with other similar bonded nonwoven sheet materials. The data are plotted and the "best-fit" lines are then drawn to illustrate the relationship between the tufted-sheet properties and the structural characteristics of the bonded nonwoven sheet materials.

## EXAMPLE 12

An isotactic polypropylene web of 4 in. (10 cm.) staple 10 fibers (8 d.p.f.) (0.9 tex) is made on a Garnett card and bonded at 78 p.s.i.a. (5.5 kg./cm.<sup>2</sup>). Fifteen percent of the fibers are 1.5 g.p.d. and the remainder, 4.0 g.p.d. A polysiloxane lubricant is applied to the bonded sheet. The tufted properties are 97 lbs. (44 kg.) grab tensile (unit weight 3.6 oz./yd.<sup>2</sup>); (122 gm./m.<sup>2</sup>) and a dye-beck-width loss of 5%. Characterization of the bonded sheet is as follows:

5 The top layer of cloth was replaced and each web section subjected to heat treatment by passage through a bonder. The webs were prepared at two different bonding temperatures as follows:

Web A 157.5° C.

Web B 159.3° C.

15 The binder concentration was calculated to be about 24% by weight. The bonded webs were lubricated and then tufted. The bond strength distribution parameters prior to tufting and tufted grab tensile values for the tufted sheets appear in Table 10 below.

TABLE 10

| Web    | Web Wt.,<br>oz./yd. <sup>2</sup> | Percent Lub<br>Pickup | TGT<br>(lbs.) | $\bar{S}$<br>(gms.) | $\sigma^2$ | $N_b\bar{S}$<br>(gms./cc.) | $N_b\bar{S}/f$<br>(cc.- <sup>1</sup> ) | TTT<br>(lbs.) |
|--------|----------------------------------|-----------------------|---------------|---------------------|------------|----------------------------|----------------------------------------|---------------|
| A----- | 4.1                              | 2.0                   | 122           | 2.7                 | 21.6       | 9.5×10 <sup>4</sup>        | 3.1×10 <sup>-1</sup>                   | 53            |
| B----- | 4.0                              | 1.9                   | 92            | 1.9                 | 19.0       | 11.1×10 <sup>4</sup>       | 3.6×10 <sup>-1</sup>                   | 44            |

TTT=Tufted Tongue Tear (machine direction); TGT=Tufted Grab Tensile (cross machine direction);  $\bar{S}$ =Average Bond Strength;  $\sigma^2$ =Variance;  $N_b$ =Number of bonds per cubic centimeter with strength greater than 0.1 gm.;  $f$ =Fiber breaking strength, grams/filament.

$$\bar{S}=1.3$$

$$\sigma^2=5.5$$

$$N_b\bar{S}=6.4\times 10^4$$

$$N_b\bar{S}/f=2.3\times 10^3$$

## EXAMPLE 13

This example illustrates the relative insensitivity of the bonded nonwoven sheets of this invention to the condition of the tufting needles. For comparison, the results obtained with nonwoven carpet backing prepared by self-bonding nonwoven webs of like continuous filaments of isotactic polypropylene are also presented. The nonwoven sheets are comparable in all respects except that the nonwoven sheet of this invention is prepared by bonding a nonwoven web of mixed-orientation polypropylene filaments while the control sheet is prepared by self-bonding the nonwoven web of polypropylene filaments all having the same level of orientation. The high-oriented filaments of the mixed-orientation web have the same level of orientation as the filaments in the control sheet. The grab-tensile strengths of bonded and lubricated nonwoven sheets after tufting with new and damaged needles are summarized below for two series of tests.

What is claimed is:

1. A bonded nonwoven sheet comprising a matrix of synthetic organic fibers having a breaking strength of at least 7 grams, said fibers being interconnected at a multiplicity of points throughout the sheet, by at least some bonds having a strength greater than 0.1 gram, the average strength of these bonds being at least 0.9 gram and less than the matrix fiber breaking strength, the said bond strength distribution being characterized by a variance of at least 4, the number of said bonds being such that the product of the number of bonds per cubic centimeter and the average bond strength is greater than  $5\times 10^4$  g./cm.<sup>3</sup> and this product divided by the fiber breaking strength is less than  $9\times 10^3$ /cm.<sup>3</sup>

2. The product of claim 1 wherein the matrix fiber is isotactic polypropylene of high orientation.

3. The product of claim 2 which additionally contains 50 polypropylene fiber of low orientation as a binder fiber.

4. The product of claim 3 wherein the matrix and binder fibers are sections along the length of single filaments.

5. The product of claim 1 wherein the fiber denier is 55 between 3 and 15.

6. A bonded nonwoven sheet comprising matrix and binder fiber, said matrix fiber being synthetic organic fibers having an average breaking strength of at least 7 grams, the fibers of the sheet being interconnected at a multiplicity of points throughout the sheet by at least some bonds having a strength greater than 0.1 gram, the average strength of said bonds being at least 0.9 gram and less than the matrix fiber breaking strength, the strength distribution of said bonds being characterized by a variance of at least 4, the number of said bonds being such that the product of the number of bonds per cubic centimeter and the average bond strength is greater than  $5\times 10^4$  g./cm.<sup>3</sup> and this product divided by the fiber breaking strength is less than  $9\times 10^3$ /cm.<sup>3</sup>

7. The product of claim 6 wherein the matrix and binder fiber are polypropylene of high and low orientation respectively.

| Needle Condition                                              | Tufted-Grab-Tensile, lb. (kg.)         |                                  |
|---------------------------------------------------------------|----------------------------------------|----------------------------------|
|                                                               | Nonwoven<br>sheet of<br>this invention | Control,<br>selfbonded-<br>sheet |
| A. All new pointed needles-----                               | 150 (68)                               | 134 (61)                         |
| One slightly burred needle-----                               | 149 (68)                               | 126 (57)                         |
| One severely burred needle-----                               | 147 (67)                               | 119 (54)                         |
| Two adjacent burred needles-----                              | 144 (65)                               | 81 (37)                          |
| Three adjacent burred needles-----                            | 143 (65)                               | 67 (30)                          |
| Two burred needles separated by<br>three pointed needles----- | 151 (69)                               | 67 (30)                          |
| B. All new pointed needles-----                               | 128 (58)                               | 155 (71)                         |
| All burred needles-----                                       | 80 (36)                                | 58 (26)                          |

## EXAMPLE 14

A random unbonded unconsolidated web of polypropylene fibers was collected between pieces of porous cloth. The fibers (9 d.p.f.) had a breaking strength of 30.5 75

3,502,538

15

8. The sheet of claim 1 wherein the synthetic organic fibers are continuous filaments.

16

FOREIGN PATENTS

808,287 2/1959 Great Britain.  
844,760 8/1960 Great Britain.

References Cited

UNITED STATES PATENTS

5

3,193,442 7/1965 Schulz et al. ----- 161—169  
3,276,944 10/1966 Levy ----- 161—170  
3,396,071 8/1968 Couzens ----- 161—170

ROBERT F. BURNETT, Primary Examiner

L. M. CARLIN, Assistant Examiner

U.S. CL. X.R.

161—170

UNITED STATES PATENT OFFICE  
CERTIFICATE OF CORRECTION

Patent No. 3,502,538 Dated 3/24/70

Inventor(s) Joseph Claine Petersen

It is certified that error appears in the above-identified patent and that said Letters Patent are hereby corrected as shown below:

- Column 5, line 49, "narow" should read --narrow--.
- Column 6, line 15, "retain" should read --remain--.
- Column 6, line 44, "machinne" should read --machine--.
- Column 6, line 71, put a period after "inches".
- Column 7, line 9, "0.38" should read --0.83--.
- Column 9, Table 6, 6th column, third number, "32.1" should read --23.1--.
- Column 10, Table 4, last column, second number, "2" should read --22--.
- Column 12, line 17, "3,790" should read --3,970--.

SIGNED AND  
SEALED

**AUG 18 1970**

**(SEAL)**

Attest:

Edward M. Fletcher, Jr.

Attesting Officer

WILLIAM E. SCHUYLER, JR.  
Commissioner of Patents